

## UNITED STATES PATENT OFFICE

2,233,103

## PRODUCTION OF NICKEL POWDER

Charles Leigh Mantell, Manhasset, N. Y., assignor  
to Hardy Metallurgical Company, New York,  
N. Y., a corporation of Delaware

No Drawing. Application April 6, 1938,  
Serial No. 200,418

11 Claims. (Cl. 204—10)

This invention relates to the production of nickel in finely divided form, and particularly to the production of nickel powder by electrolytic deposition from a solution.

5 It has been customary heretofore to plate nickel out of solution in massive form, employing acidified aqueous baths of nickel salt. Efforts to produce a finely divided deposit of nickel by electrolysis of such baths have not been successful, 10 the nickel tending to deposit in massive form even at relatively high current density, so that heretofore nickel powders have been produced by pyrometallurgical processes, usually from nickel carbonyl.

15 However, as a result of my investigations, I have discovered a method of depositing nickel in finely divided form, which method is simple and reliable, does not require excessive current densities or excessive power consumption and employs an inexpensive electrolyte. In the practice of my invention, I employ an alkaline aqueous solution containing nickel in the form of nickel-ammonium ions, and endeavor to maintain the concentration of true nickel ions in the solution 25 at a minimum.

In brief, the method of my invention for producing nickel in finely divided form comprises subjecting to electrolysis in an electrolytic cell containing an anode and a cathode, an alkaline aqueous solution consisting essentially of alkali ions, nickel-ammonium ions, hydroxyl ions and chloride ions, whereby the nickel tends to deposit at the cathode in powder form or in a condition in which it is easily reduced to powder 30 form. As indicated hereinbefore, it is desirable to maintain the proportion of nickel-ammonium ions to nickel ions in the solution relatively high during electrolysis.

35 In the presently preferred practice of my invention, the operation is begun with an electrolyte in the form of an alkaline aqueous solution of ammonium chloride. A soluble nickel bearing anode is employed so that the nickel tends to dissolve therefrom and enter the solution in the 40 form of the nickel-ammonium complex. The nickel deposits from the solution in finely-divided form at a cathode, which preferably is made of sheet nickel.

45 I prefer to employ an ammonium chloride solution containing at least 200 grams per liter of ammonium chloride. However, saturated solutions of ammonium chloride may be employed, the saturation point for ammonium chloride at 0° C. 50 being 297 grams per liter. At a temperature of

20° C., the bath may contain as much as 300 grams per liter of ammonium chloride.

The bath must be alkaline and the alkalinity preferably is obtained by adding from 1 to 3 grams per liter of sodium hydroxide or its equivalent. 5 The temperature of the bath should range from 20 to 30° C. for best results. The nickel anode may be cast or electrolytically deposited metal. Anode current densities may vary from as low as 10 amperes per square foot to as high as 60 amperes per square foot. For the sake of electrical economy, anode current densities of from 10 to 20 amperes per square foot are preferred.

10 The cathode preferably should be of smooth sheet nickel and cathode current densities may 15 vary from 20 to 120 amperes per square foot. However, cathode current densities of the order of 20 to 30 amperes per square foot are preferred.

20 In operation, the bath preferably should contain substantially no nickel ions and at all times 20 the nickel ion concentration should be kept low. A low concentration of nickel ions in the solution may be obtained by adjusting the relationship between the current density at the anode and the current density of the cathode so that 25 the nickel deposits at the cathode at substantially the same rate and at worst, at only a slightly lower rate than it goes into the solution at the anode.

30 Due to the presence of the nickel-ammonium complex in the electrolyte, it attains a blue color. In practice proper concentration of nickel-ammonium ions in the solution can be judged by the color thereof. In the event that a substantial concentration of nickel ions tends to develop in 35 the electrolyte (and this may be determined either through a change in the color of the electrolyte or by chemical analysis) it is desirable to decrease the rate of anode corrosion. This is done conveniently by introducing insoluble anodes into 40 the bath along with the nickel bearing anodes. Thus, carbon or graphite electrodes may be used for insoluble anodes. By increasing the ratio of exposed surface of insoluble anodes to the exposed surface of soluble nickel anodes in the 45 bath, it is possible to decrease the rate of solution of nickel at the anode to a point where the deposition rate at the cathode exceeds it. In this way, the tendency of the nickel to build up in solution and ionize as nickel ions instead of 50 nickel-ammonium ions, is overcome.

55 At the preferred anode and cathode current densities, i. e., an anode current density of 10 to 20 amperes per square foot and a cathode current density in excess of 20 amperes per square 55

foot, the electrolyte (which originally is colorless and contains no nickel) assumes a light blue shade due to the formation of the nickel-ammonium complex. The nickel-ammonium complex salt in the solution has very little tendency to form nickel ions because the primary ionization of the salt produces ammonium ions, and only a secondary ionization (taking place to a much smaller extent than the first) produces nickel ions.

In operation, under the conditions hereinbefore prescribed, the powdery deposit of nickel formed at the cathode is relatively adherent so that the cathode may be lifted out of the solution without disturbing the deposit. The deposit may be then removed from the cathode by flushing, washing or scraping after which the cathode may be returned to the cell. The powdery deposit is freed from all electrolyte by water washing, then physically separated from the water by any of the conventional methods such as filtration, centrifuging, decanting and the like, and thereafter dried and subjected to slight crushing to reduce any large aggregates.

If, during the washing operation, oxidation products have been formed on the surface of the powder particles, these may be reduced by the action of a reducing gas at a high temperature, for example, hydrogen. Following drying and any necessary reduction operation, the powder may be ground and sized for various industrial applications.

Grinding and sizing may take place while the product is in a wet condition. Thus, in the wet condition, sizing may be accomplished by elutriation or any of the other customary methods of hydraulic classification.

The practice of my invention will be more thoroughly understood in the light of the following detailed description of a presently preferred practice, taken in conjunction with the accompanying table which shows the conditions pertaining to the operation and the results obtained.

cell an aqueous solution containing 300 grams per liter of ammonium chloride and 2 grams per liter of sodium hydroxide. An anode of electrolytically deposited nickel was placed in the cell in contact with the electrolyte, the cathode being a piece of pure sheet nickel. Direct current was passed through the cell under the conditions indicated in the table and in all instances nickel deposited at the cathode in the form of a very fine powder. A small amount of the nickel powder tended to slough off the cathode and deposit in the bottom of the tank. In Test I, the deposit at the cathode was very easy to remove, the cathode current density in this instance being 20 amperes per square foot. At higher current densities, i. e., in Tests II, III, IV, V and VI, the powder deposit tended to adhere more firmly to the cathode and it was noted that as the current density was increased, it was correspondingly harder to remove the powder deposit from the cathode. It will be noted that in Test I, operating at a current density of 20 amperes per square foot, the lowest voltage was obtained together with the maximum deposit. Moreover, the deposit obtained in Test No. I was more easily ground than the deposit obtained in other instances.

It is not essential that the nickel ammonium complex ions be obtained through solution of a soluble nickel anode. Thus, for example, it is possible to obtain a satisfactory deposit of nickel powder by carrying on the electrolysis of the solution of the complex nickel ammonium salt however this salt be derived.

I claim:

1. A method of producing nickel in finely divided form which comprises subjecting to electrolysis in an electrolytic cell in the presence of a cathode and a nickel-bearing anode, an alkaline aqueous solution consisting essentially of alkali ions, nickel-ammonium ions, hydroxyl ions, and chloride ions whereby the nickel tends to be dis-

| 45                                       |                         | Test No. |         |         |         |         |         | 45 |
|------------------------------------------|-------------------------|----------|---------|---------|---------|---------|---------|----|
|                                          |                         | I        | II      | III     | IV      | V       | VI      |    |
| 50                                       | Date                    | 1/12/38  | 1/12/38 | 1/12/38 | 1/12/38 | 1/12/38 | 1/12/38 | 50 |
| Electrolyte:                             |                         |          |         |         |         |         |         |    |
| Ammonium chloride.....                   | grams per liter         | 300      | 300     | 300     | 300     | 300     | 300     |    |
| Sodium hydroxide.....                    | do                      | 2        | 2       | 2       | 2       | 2       | 2       |    |
| Volume of electrolyte.....               |                         | 2000     | 2000    | 2000    | 2000    | 2000    | 2000    |    |
| Total current.....                       | amperes                 | 3.12     | 3.12    | 3.12    | 3.12    | 3.12    | 3.12    |    |
| Voltage.....                             | average                 | 1.45     | 1.51    | 1.49    | 1.62    | 1.62    | 1.72    |    |
| Anode material.....                      |                         |          |         |         |         |         |         |    |
| No. of anodes.....                       |                         | 2        | 2       | 2       | 2       | 2       | 2       |    |
| Anode area.....                          | square inches           | 43.2     | 21.6    | 14.4    | 10.8    | 8.6     | 7.2     | 55 |
| Anode current density.....               | amperes per square foot | 10       | 20      | 30      | 40      | 60      | 60      |    |
| Original weight of anodes.....           | grams                   | 1654.5   | 778.0   | 407.5   | 429.5   | 445.0   | 338.0   |    |
| Final weight of anodes.....              | do                      | 1635.5   | 768.5   | 389.0   | 410.0   | 426.0   | 319.0   |    |
| Anode weight loss.....                   | do                      | 19.0     | 19.5    | 18.5    | 19.5    | 19.0    | 19.0    |    |
| Cathode material.....                    |                         |          |         |         |         |         |         |    |
| No. of cathodes.....                     |                         | 1        | 1       | 1       | 1       | 1       | 1       |    |
| Cathode area.....                        | square inches           | 21.6     | 10.8    | 7.2     | 5.4     | 4.3     | 3.6     | 60 |
| Cathode current density.....             | amperes per square foot | 20       | 40      | 60      | 80      | 100     | 120     |    |
| Original weight of cathodes.....         | grams                   | 16.8     | 11.4    | 8.1     | 9.5     | 11.3    | 11.3    |    |
| Final weight of cathodes.....            | do                      | 29.2     | 23.3    | 12.9    | 18.0    | 20.7    | 20.6    |    |
| Cathode weight gain.....                 | do                      | 12.4     | 11.9    | 4.8     | 8.5     | 9.4     | 9.3     |    |
| Weight of Ni powder in tank.....         | do                      | 1.0      | 6       | 5.1     | 1.8     | 1.0     | 1.3     |    |
| Total weight of Ni.....                  | do                      | 13.4     | 12.5    | 9.9     | 10.3    | 10.4    | 10.6    |    |
| Anode-cathode distance.....              | inches                  | 1.5      | 1.5     | 1.5     | 1.5     | 1.5     | 1.5     | 65 |
| Temperature of electrolyte at start..... | ° C                     | 23.5     | 24      | 24      | 23      | 24      | 24      |    |
| Time of electrolysis.....                | hours                   | 7        | 7       | 7       | 7       | 7       | 7       |    |
| Current efficiency.....                  | percent                 | 56.0     | 52.3    | 41.4    | 43.1    | 43.5    | 43.9    |    |
| Kilowatt-hr. per pound of Ni.....        | do                      | 1.05     | 1.13    | 1.57    | 1.41    | 1.61    | 1.56    |    |
| Pounds of Ni per kw.-hr.....             | do                      | .95      | .88     | .64     | .71     | .62     | .64     |    |
| Percent Ni.....                          |                         | 97.47    |         |         |         |         |         |    |

70 Type deposit: The deposit in all cases was in the form of a very fine powder on the cathode with very little deposit in the bottom of the tank. The deposit in Test No. I was very easy to remove. It was noted that as the C. D. was increased (Tests II to VI) it was correspondingly harder to remove the deposit.

Remarks: It is to be noted that Test I, running at the lowest C. D., used the least voltage and gave the maximum deposit. Furthermore, this deposit was the easiest to grind.

In the examples reported in the table, the operation was started by placing in an electrolytic

solved from the anode and deposited at the cathode in finely divided form.

2. A method of producing nickel in finely divided form which comprises subjecting to electrolysis in an electrolytic cell in the presence of a cathode and a nickel-bearing anode, an alkaline aqueous solution containing originally at least 5 200 grams of ammonium chloride per liter and consisting essentially of alkali ions, nickel-ammonium ions, hydroxyl ions, and chloride ions.
3. A method of producing nickel in finely divided form which comprises subjecting to electrolysis in an electrolytic cell in the presence of a cathode and a nickel-bearing anode, an alkaline aqueous solution containing originally at 10 15 least 200 grams of ammonium chloride per liter and consisting essentially of alkali ions, nickel-ammonium ions, hydroxyl ions, and chloride ions, and maintaining a cathode current density of at least 20 amperes per square foot.
4. A method of producing nickel in finely divided form which comprises subjecting to electrolysis in an electrolytic cell in the presence of a cathode and a nickel-bearing anode, an alkaline aqueous solution containing at least originally 20 25 from 200 to 300 grams per liter of ammonium chloride and consisting essentially of alkali ions, nickel-ammonium ions, hydroxyl ions, and chloride ions, and maintaining a cathode current density of at least 20 amperes per square foot.
5. A method of producing nickel in finely divided form which comprises subjecting to electrolysis in an electrolytic cell in the presence of a cathode and a nickel-bearing anode, an alkaline aqueous solution consisting essentially of alkali ions, nickel-ammonium ions, hydroxyl ions, and chloride ions, the alkalinity of which solution is equivalent to from 1 to 3 grams of sodium hydroxide per liter and containing at least originally 30 35 from 200 to 300 grams per liter of ammonium chloride and maintaining a cathode current density of at least 20 amperes per square foot.
6. A method of producing nickel in finely divided form which comprises subjecting to electrolysis in an electrolytic cell in the presence of a cathode and a nickel-bearing anode, an alkaline aqueous solution containing at least originally 40 45 from 200 to 300 grams per liter of ammonium chloride and consisting essentially of alkali ions, nickel-ammonium ions, hydroxyl ions, and chloride ions, maintaining a cathode current density of from 20 to 120 amperes per square foot and maintaining an anode current density of from 10 to 20 amperes per square foot.
7. A method of producing nickel in finely divided form which comprises subjecting to electrolysis in an electrolytic cell in the presence of a cathode and a nickel-bearing anode, an alkaline aqueous solution containing at least originally 50 55 from 200 to 300 grams per liter of ammonium chloride and consisting essentially of alkali

ions, nickel-ammonium ions, hydroxyl ions, and chloride ions, maintaining the temperature of the electrolyte at from 20 to 30° C., and maintaining a cathode current density of from 20 to 120 amperes per square foot.

8. A method of producing nickel in finely divided form which comprises subjecting to electrolysis in an electrolytic cell in the presence of a cathode and a nickel-bearing anode, an alkaline aqueous solution containing at least originally 10 from 200 to 300 grams per liter of ammonium chloride and consisting essentially of alkali ions, nickel-ammonium ions, hydroxyl ions, and chloride ions, maintaining a cathode current density of at least 20 amperes per square foot 15 and regulating the ratio of the anode surface in contact with the solution to the cathode surface in contact with the solution so that nickel deposits at the cathode at substantially the same rate that it goes into solution at the anode. 20

9. A method of producing nickel in finely divided form which comprises subjecting to electrolysis in an electrolytic cell in the presence of a cathode and in the presence of an insoluble anode and a nickel-bearing anode, an alkaline aqueous solution containing at least originally 25 from 200 to 300 grams per liter of ammonium chloride and consisting essentially of alkali ions, nickel-ammonium ions, hydroxyl ions, and chloride ions, maintaining a cathode current density 30 of at least 20 amperes per square foot and regulating the rate at which the nickel goes into solution at the anode by regulating the ratio of the exposed surface of the nickel-bearing anode to the exposed surface of the insoluble anode. 35

10. A method of producing nickel in finely divided form which comprises subjecting to electrolysis in an electrolytic cell in the presence of a cathode and a nickel-bearing anode, an alkaline aqueous solution containing at least originally 40 from 200 to 300 grams per liter of ammonium chloride and consisting essentially of alkali ions, nickel-ammonium ions, hydroxyl ions, and chloride ions, maintaining a cathode current density of at least 20 amperes per square foot 45 during electrolysis, and maintaining a relatively high ratio of nickel-ammonium ions to nickel ions in said solution during electrolysis.

11. A method of producing nickel in finely divided form which comprises subjecting to electrolysis in an electrolytic cell having a cathode therein an alkaline aqueous solution of ammonium chloride consisting essentially of alkali ions, nickel ions, nickel-ammonium ions, hydroxyl ions, and chloride ions, and maintaining the proportion of nickel-ammonium ions to nickel ions 50 55 in said solution relatively high during electrolysis, whereby the nickel tends to deposit at the cathode in finely divided form.

CHARLES LEIGH MANTELL. 60